

## UNITED STATES PATENT OFFICE

2,551,170

COBALT BASE ALLOY AND ARTICLES  
THEREOF

Robert A. Schmucker, Jr., East Orange, Charles D. Preusch, Orange, and Lloyd F. Bowne, Jr., East Orange, N. J., assignors to Crucible Steel Company of America, New York, N. Y., a corporation of New Jersey

No Drawing. Application September 30, 1947,  
Serial No. 777,106

4 Claims. (Cl. 75—171)

1

This invention pertains to cobalt-base, cast alloys containing carbon, chromium and metal of the group tungsten and molybdenum as essential constituents, and such as are primarily adapted for cutting tools, particularly of the "high speed" variety, and which are also adapted for other wear- and abrasion-resisting applications, for example dies.

For a number of years past, cast alloy cutting tools consisting basically of the above-mentioned elements have been used for machining at greater speed than is possible with high speed steels. In order to secure even greater cutting properties, other elements, such as boron, vanadium, tantalum and columbium, have been added to the basic cobalt-chromium-carbon-tungsten and/or molybdenum cast alloys aforesaid. Cutting tools containing one or more of these additional elements are now widely used commercially.

The two principal requirements of a cobalt-base, cast alloy cutting tool of this type are: (1) that it must have sufficient wear or "cratering" resistance at elevated temperatures, to accomplish cutting at high speeds for a maximum length of time; and (2) it must have sufficient toughness to resist, under unfavorable conditions, chipping of the cutting edge or breaking of the tool bit itself. Carbon, boron, tungsten and chromium are among those elements which, while contributing to wear-resistance or general cutting life of the tool, can not be present in excessive percentages without producing an alloy which is too brittle.

In order to obtain a cobalt-base, cast cutting alloy having a composition possessing the above required characteristics, most of the commercial cast cutting alloys of the type under consideration have been of analyses such as to fall within, or nearly within, the following percentage limits as regards the basic constituents, viz.:

| C   | Cr   | W    | Co   | B   |
|-----|------|------|------|-----|
| 1.0 | 25.0 | 12.0 | 36.0 | 0   |
| 2.5 | 35.0 | 20.0 | 46.0 | 1.5 |

Now we have discovered, in accordance with a basic concept of the present invention, that an improvement in cutting life, amounting to about 25% as compared to the results obtainable with the commercial alloys aforesaid, may be obtained by the employment in cobalt-base, cast cutting alloys of this character, of chromium in excess of 35%, i. e., within the range of about 35.5 to 40% and preferably 35.5 to 38%, in conjunction with metal of the group tungsten and molybdenum

2

within a restricted range of about 14 to 20% and preferably 16 to 19%, and boron in excess of 0.5, i. e., about 0.6 to 1.5% and preferably about 0.7 to 1%. In so far as we are aware, cobalt-base, cast cutting alloys within this range of analysis have never heretofore been produced commercially, or known to those skilled in the art, nor have the superior cutting qualities thereof been heretofore pointed out or suggested.

Although either tungsten or molybdenum or both may be employed within the limits set forth in the above range of analysis for the present invention, tungsten is ordinarily preferred. Also, within these limits, the tungsten content should be decreased as the chromium content is increased, or vice versa, in order to avoid undue brittleness in the resulting alloy.

The carbon content of alloys in accordance with the invention should lie within the range of about 1 to 3%, and preferably about 1.5 to 2.5%. Carbon contents above about 2% generally produce heats with better results in log turning tests than do lower carbon heats. Boron contents over about 0.6% increase this tendency.

The qualities of alloys in accordance with the invention, when employed as cutting tools, are further improved by additions of other elements as follows:

Vanadium improves the toughness and the cutting properties of the alloy, and to this end should be present within broad limits of about 1.5 to 6%, and narrower limits of about 3 to 5%, vanadium of over 4% being preferred.

Nickel increases the toughness and decreases the hardness of the alloy, and hence may be added for this purpose in amounts up to about 10%, and more preferably up to about 6%, excellent results being obtainable with about 3% nickel. These same remarks apply to iron, which may be added within these same broad, preferred and recommended percentages.

Additions of nitrogen to the alloy in excess of about 0.1% and up to about 0.25% increase the cutting life of the alloy, and hence is a useful constituent of preferred analyses in accordance with the present invention. To this end, nitrogen may advantageously be added within the range of about 0.1 to 0.25% by weight of the resulting alloy.

Molybdenum, tungsten and chromium, in that order, are the most potent hardeners of the alloy and it is for this reason that increases in chromium within the range of the present invention must be accompanied by corresponding reductions in the amounts of molybdenum and tungsten, or vice versa. On the other hand, nitrogen, boron, carbon and vanadium appear to have

only a slight effect on hardness within the range of analysis covered by the present invention. Nickel and iron, partially replacing cobalt, decrease hardness in that order.

Although manganese and silicon appear to have no particular advantageous or deleterious effects on the alloy, when present in small amounts, they are ordinarily unavoidably present to some extent, but should be held within limits of about 1.5% each maximum, and the manganese should preferably be limited to about 0.5% and the silicon to about 1%.

Aside from the required and optional additions to the alloy above outlined, the balance thereof will be substantially cobalt.

A broad range of analysis for cobalt-base, cast

By way of demonstrating the superiority of cast cobalt-base cutting alloys in accordance with the present invention, as compared to previously known and used alloys of this type, comparative cutting test results thereon are submitted in the following Table I. These cutting tests, the results of which are given in Table I, were for groups I-III carried out on an annealed chromium-nickel round log, approximating 15" in diameter, at a speed of 135 surface feet per minute, using a feed of 0.045" per revolution and a cutting depth of  $\frac{1}{16}$ ". The cutting tests in group IV of Table I were carried out on a similar log of somewhat higher hardness at a speed of 110 surface feet per minute, using a feed of 0.040" per revolution and a cutting depth of  $\frac{1}{16}$ ".

Table I

| Alloy                                | Chemical Analysis, Percent |         |         |           |           |         |         |          |      |      |         | Hardness Rockwell "C" | Cutting Time to Failure, Min. (Average two or more tools) |       |
|--------------------------------------|----------------------------|---------|---------|-----------|-----------|---------|---------|----------|------|------|---------|-----------------------|-----------------------------------------------------------|-------|
|                                      | C                          | B       | N       | Cr        | W         | Mo      | V       | Ni       | Fe   | Mn   | Si      |                       |                                                           |       |
| GROUP I—EFFECT OF VARYING CHROMIUM   |                            |         |         |           |           |         |         |          |      |      |         |                       |                                                           |       |
| A                                    | 1.4/2.0                    | .75/.90 | .10/.15 | 29.5/32.0 | 17.9/20.0 | .40/.70 | 3.8/4.5 | .20/3.50 | 13.0 | 0.10 | .10/.40 | Bal...                | 60/63                                                     | 8.55  |
| B                                    | 2.06                       | 0.90    | 0.11    | 31.75     | 16.84     | 0.51    | 3.93    | 3.32     | 2.67 | 0.10 | 0.32    | Bal...                | 59/61.5                                                   | 9.51  |
| C                                    | 2.07                       | 0.84    | 0.13    | 34.59     | 16.24     | 0.55    | 4.12    | 2.96     | 2.71 | 0.07 | 0.28    | Bal...                | 59.5/62                                                   | 9.98  |
| D                                    | 2.19                       | 0.76    | 0.15    | 35.70     | 16.62     | 0.62    | 4.01    | 3.16     | 2.04 | 0.07 | 0.52    | Bal...                | 60/61.5                                                   | 12.04 |
| E                                    | 2.12                       | 0.86    | 0.15    | 36.25     | 16.24     | 0.60    | 4.09    | 3.16     | 2.11 | 0.07 | 0.40    | Bal...                | 61/62                                                     | 13.05 |
| GROUP II—EFFECT OF VARYING TUNGSTEN  |                            |         |         |           |           |         |         |          |      |      |         |                       |                                                           |       |
| F                                    | 2.13                       | 0.76    | 0.15    | 36.30     | 10.92     | 0.51    | 4.08    | 3.04     | 1.69 | 0.09 | 0.38    | Bal...                | 58.5/60.5                                                 | 8.40  |
| G                                    | 2.13                       | 0.79    | 0.15    | 35.85     | 14.00     | 0.58    | 4.21    | 3.06     | 1.87 | 0.07 | 0.32    | Bal...                | 59.5/61.5                                                 | 9.85  |
| H                                    | 2.12                       | 0.86    | 0.15    | 36.25     | 16.24     | 0.60    | 4.09    | 3.16     | 2.11 | 0.07 | 0.40    | Bal...                | 61/62                                                     | 13.05 |
| I                                    | 2.19                       | 0.79    | 0.16    | 36.00     | 17.14     | 0.58    | 4.16    | 3.30     | 1.99 | 0.06 | 0.40    | Bal...                | 61/63                                                     | 13.80 |
| J                                    | 2.16                       | 0.79    | 0.17    | 36.00     | 19.60     | 0.58    | 4.09    | 3.04     | 1.62 | 0.08 | 0.32    | Bal...                | 63/64.5                                                   | 15.00 |
| GROUP III—EFFECT OF VARYING NITROGEN |                            |         |         |           |           |         |         |          |      |      |         |                       |                                                           |       |
| K                                    | 2.15                       | 0.81    | 0.05    | 36.04     | 16.92     | 0.55    | 4.05    | 3.00     | 1.63 | 0.08 | 0.38    | Bal...                | 60.5/62.5                                                 | 10.87 |
| L                                    | 2.10                       | 0.84    | 0.09    | 36.05     | 16.78     | 0.57    | 4.23    | 3.32     | 1.89 | 0.08 | 0.32    | Bal...                | 61/62.5                                                   | 10.95 |
| M                                    | 2.07                       | 0.90    | 0.14    | 36.75     | 16.48     | 0.62    | 4.27    | 3.20     | 2.18 | 0.08 | 0.44    | Bal...                | 62                                                        | 12.00 |
| N                                    | 2.16                       | 0.88    | 0.14    | 35.52     | 17.04     | 0.67    | 4.11    | 3.40     | 2.44 | 0.06 | 0.46    | Bal...                | 63                                                        | 12.00 |
| O                                    | 2.25                       | 0.79    | 0.18    | 36.20     | 16.96     | 0.60    | 4.03    | 3.26     | 1.88 | 0.03 | 0.36    | Bal...                | 61/62                                                     | 15.15 |
| P                                    | 2.12                       | 0.79    | 0.19    | 36.35     | 16.18     | 0.66    | 4.11    | 3.24     | 2.26 | 0.10 | 0.36    | Bal...                | 60/62                                                     | 12.15 |
| GROUP IV—EFFECT OF VARYING BORON     |                            |         |         |           |           |         |         |          |      |      |         |                       |                                                           |       |
| Q                                    | 1.84                       | 0.34    | 0.15    | 36.60     | 16.40     | 0.47    | 4.10    | 3.00     | 0.85 | 0.06 | 0.38    | Bal...                | 60                                                        | 4.01  |
| R                                    | 1.97                       | 0.48    | 0.16    | 36.25     | 16.36     | 0.51    | 4.17    | 3.00     | 0.96 | 0.06 | 0.36    | Bal...                | 61/63                                                     | 9.00  |
| S                                    | 2.18                       | 0.75    | 0.16    | 35.95     | 16.88     | 0.66    | 4.01    | 3.20     | 1.95 | 0.12 | 0.44    | Bal...                | 59/61                                                     | 11.30 |
| T                                    | 2.07                       | 0.95    | 0.15    | 36.59     | 16.20     | 0.64    | 4.17    | 3.20     | 1.28 | 0.07 | 0.28    | Bal...                | 61/62                                                     | 13.0  |

<sup>1</sup> Maximum.

cutting alloys in accordance with the invention will be as follows:

| Element             | Per cent  |
|---------------------|-----------|
| Carbon              | 1.0-3.0   |
| Boron               | 0.6-1.5   |
| Chromium            | 35.5-40.0 |
| Tungsten-Molybdenum | 14.0-20.0 |
| Vanadium            | 1.5-6.0   |
| Iron                | 0-10.0    |
| Nickel              | 0-10.0    |
| Manganese           | 0-1.5     |
| Silicon             | 0-1.5     |
| Cobalt              | Remainder |

A narrower and more preferred range of analysis is as follows:

| Element             | Per cent  |
|---------------------|-----------|
| Carbon              | 1.5-2.5   |
| Boron               | 0.7-1.0   |
| Chromium            | 35.5-38.0 |
| Tungsten-Molybdenum | 16.0-19.0 |
| Vanadium            | 3.0-5.0   |
| Iron                | 0-6.0     |
| Nickel              | 0-6.0     |
| Manganese           | 0-0.5     |
| Silicon             | 0-1.0     |
| Cobalt              | Remainder |

From the group I tests in the above table, it will be seen that the previously known or used alloys A, B and C are definitely inferior, as regards cutting tests, to alloys D and E in accordance with the present invention. Similarly, in the group II tests, alloy F containing chromium within the range of the present invention but containing tungsten below the range, is definitely inferior to alloys G, E, I and J, the latter containing both chromium and tungsten within applicants' range. The group III tests establish that for alloys in accordance with the present invention, superior results are obtained by adding thereto nitrogen in excess of about 0.10 and up to about 0.25%, as is evidenced by comparison of the cutting test results for alloys K and L containing nitrogen below this range, with the results obtained for alloys M, N, O and P containing nitrogen within this range. Likewise, the group IV tests establish that for alloys Q and R containing chromium and tungsten with in the ranges of the present invention, but containing boron outside the range, i. e., below about 0.6%, that materially lower cutting times to failure are obtained than is the case of alloys S and T containing boron within the range of the present invention of 0.6 to 1.5%.

From the group I test results given in Table I, a chromium content of about 36% was selected as best, for alloys in accordance with the present invention, since alloys D and E gave the longest cutting times. Similarly, from the group II test results, an accompanying tungsten content of about 17% was selected, as giving the best combination of cutting properties, hardness and toughness, based on the results of alloys H and I. Although alloy J with 19.6% tungsten had a slightly better cutting value, its hardness was somewhat higher and its impact strength somewhat lower than was considered satisfactory for commercial use.

Based on these observations, approximately fifty heats having the optimum chromium and tungsten contents of about 36% and 17% respectively as aforesaid, were melted up, cast into tools, and tested, along with tools of one of the best existing commercial alloys of this type, with results as set forth in Table II below:

Table II

| Tool Type                              | Chemical Analysis, Per Cent |      |      |      |      |      |      |           | Cutting Time to Failure, (minutes) |
|----------------------------------------|-----------------------------|------|------|------|------|------|------|-----------|------------------------------------|
|                                        | C                           | B    | Cr   | W    | V    | Fe   | Ni   | Co        |                                    |
| Commercial Alloy-----                  | 1.4                         | 0.75 | 29.0 | 17.9 | 3.80 | 3.0  | 0.20 | 36.0      | 12.8 (Av.)                         |
|                                        | 2.0                         | 0.90 | 32.0 | 20.4 | 4.50 | Max. | 3.50 | 38.0      |                                    |
| Test Heats Representing the Invention. | 1.9                         | 0.75 | 35.5 | 16.0 | 3.75 | 3.0  | 3.00 | Remainder | 16.4 (Av.)                         |
|                                        | 2.3                         | 0.95 | 37.0 | 17.5 | 4.25 | Max. | 3.50 |           |                                    |

Test Conditions—Speed 110/130 SFM; Feed 0.045"/Rev.; Depth of Cut  $\frac{3}{16}$ "; Log: Annealed Chromium-Nickel Steel.

The improved cutting properties of cast cobalt-base cutting alloys in accordance with the present invention are thus clearly demonstrated by the results set forth in the above Tables I and II.

We claim:

1. A cast cutting alloy having substantially the following composition: 35.5 to 40% chromium; 14 to 20% of metal of the group tungsten and molybdenum, the metal of said group being substantially inversely proportional to the chromium content; 1 to 3% carbon; 0.6 to 1.5% boron; 1.5 to 6% vanadium; up to 10% each of iron and nickel; up to 1.5% each of manganese and silicon; and the balance cobalt.

2. A cast cutting alloy having substantially the following composition: 35.5 to 38% chromium; 16 to 19% of metal of the group tungsten and molybdenum, the metal of said group being substantially inversely proportional to the chromium content; 1.5 to 2.5% carbon; 0.7 to 1% boron; 3 to 5% vanadium; up to 6% each of iron

and nickel; up to 0.5% manganese; up to 1% silicon; and the balance cobalt.

3. A cast cutting alloy having substantially the following composition: 35.5 to 40% chromium; 14 to 20% of metal of the group tungsten and molybdenum, the metal of said group being substantially inversely proportional to the chromium content; 1 to 3% carbon; 0.6 to 1.5% boron; 1.5 to 6% vanadium; up to 10% each of iron and nickel; up to 1.5% each of manganese and silicon; 0.10 to 0.25% nitrogen; and the balance cobalt.

4. A cast cutting alloy having substantially the following composition: 35.5 to 38% chromium; 16 to 19% of metal of the group tungsten and molybdenum, the metal of said group being substantially inversely proportional to the chromium content; 1.5 to 2.5% carbon; 0.7 to 1% boron; 3 to 5% vanadium; up to 6% each of iron and nickel; up to 0.5% manganese; up to

1% silicon; 0.1 to 0.25% nitrogen; and the balance cobalt.

ROBERT A. SCHMUCKER, JR.  
CHARLES D. PREUSCH.  
LLOYD F. BOWNE, JR.

## REFERENCES CITED

The following references are of record in the file of this patent:

## UNITED STATES PATENTS

| Number    | Name                 | Date          |
|-----------|----------------------|---------------|
| 1,698,935 | Chesterfield -----   | June 15, 1929 |
| 2,030,343 | Wissler -----        | Feb. 11, 1936 |
| 2,297,687 | Burgess et al. ----- | Oct. 6, 1942  |
| 2,309,371 | Wissler -----        | Jan. 26, 1943 |
| 2,432,618 | Franks et al. -----  | Dec. 16, 1947 |

## OTHER REFERENCES

55 Progress Report on "Heat Resisting Metals for Gas Turbine Parts" (N-102), P. B. No. 39,579; September 21, 1943, stamped: "Declassified to open February 18, 1946"; page 6.